

Patented Oct. 20, 1925.

1,557,844

# UNITED STATES PATENT OFFICE.

CARL IMMERHEISER, OF LUDWIGSHAFEN-ON-THE-RHINE, AND HUGO WOLFF, OF MANNHEIM, GERMANY, ASSIGNEES, BY MESNE ASSIGNMENTS, TO BADISCHE ANILIN & SODA FABRIK, OF LUDWIGSHAFEN-ON-THE-RHINE, BAVARIA, GERMANY, A CORPORATION OF THE GRAND DUCHY OF BADEN.

## TANNING COMPOSITION.

No Drawing.

Application filed July 9, 1920. Serial No. 395,127.

To all whom it may concern:

Be it known that we, CARL IMMERHEISER and HUGO WOLFF, citizens of the German Empire, residing at Ludwigshafen-on-the-Rhine and Mannheim, respectively, Germany, have invented new and useful Improvements in Tanning Composition, of which the following is a specification.

Synthetic compounds of different kinds have recently been suggested for tanning purposes. Thus, for example, sulfonic acids of crude anthracene, crude carbazol or anthracene waste, in all save the color produced, give valuable results if employed for tanning skins or hides. The color of the leather produced is however so objectionable as to have practically precluded such leather from becoming commercial. This color is a dark brown of dull or grayish hue so different from that of leather tanned with vegetable-tanning agents as not to have gone into use either alone or in admixture therewith.

By the tanning agent below described we have succeeded in producing, within a small fraction of the time required by vegetable agents, leather tanned of the clear brown hues characteristic of the latter. To an expert in the art the difference in kind of color from that first referred to is such as to have proved vital to commercial success either when our tanning agent is used alone or in combination with a vegetable tanning agent.

It has been found that the said sulfonation product of "crude anthracene," including crude products of anthracene or of carbazol or anthracene waste and comprising, generally speaking, varying mixtures of higher hydrocarbons and of carbazol, can also be prepared in a form giving a far lighter colored leather and being therefore of an increased value. The new tanning composition can be prepared by treating the sulfonation product of "crude anthracene" with a clearing agent. For example, chlorin or a hypochlorite may be added to the crude sulfonation product, or oxalic acid may be added either to the raw product or to the preparation obtained by the action of chlorin, or hypochlorite. Formaldehyde may also be employed. Another way of obtaining the new form of the tanning preparation consists in sulfonating the initial ma-

terial with chloro-sulfonic acid instead of with sulfuric acid. The chloro-sulfonic acid can be employed at a moderate temperature and diluting means, such e. g. as nitrobenzene may be used along with it. If desired, the products obtained with chloro-sulfonic acid may also be treated with a clearing agent of the aforementioned kind. The product obtained in one way or the other is distinguished by the following reactions. When hide is suspended for several days in its acidulated solution, it assumes a pure brown color in comparison with which the coloration produced with ordinary sulfonated crude anthracene is a dull, intensely grayish brown.

The product can be employed in the usual way in a slightly acid aqueous solution, preferably together with natural tanning extracts.

In order to further illustrate the nature of the invention, the following example is given to which, however, the invention is not confined. The parts are by weight.

### Example 1.

An anthracene waste having the approximate composition: 60 per cent carbazol, 10 per cent anthracene, 20 per cent phenanthrene, 10 per cent fluorene and similar hydrocarbons is heated, to from 100 to 130 degrees centigrade, with concentrated sulfuric acid, in the proportion of 10 parts of the former to 12 parts of the latter, until the product is substantially soluble in water. The product is suitably diluted, freed from unaltered sulfuric acid by treating with lime, filtered and neutralized with soda lye. The solution of the sodium salt is then treated with sodium hypochlorite, while hot, or chlorin is introduced into the solution until its color is no longer improved, while the solution is kept neutral, or slightly alkaline by gradually adding the required amount of caustic soda lye.

### Example 2.

100 parts of crude anthracene, or of anthracene waste (residue from the purification of crude anthracene), or other mixtures of higher tar hydrocarbons, or carbazol are

suspended in 200 parts of nitrobenzene, or other suitable diluting agent, and 120 to 140 parts of chlorosulfonic acid are next introduced at temperatures below 100 degrees centigrade. Stirring is continued for some hours until the product is entirely soluble in water. Then the diluting agent is blown off with steam, or distilled off in vacuo; the solution of the sulfonic acid mixture either wholly or partly neutralized can now serve for tanning.

Oxalic acid may be added to the sulfonation products either directly or after the treatment with chlorin or hypochlorite, as described in the foregoing example, in the proportion of say 20 to 40 parts to every 100 parts of initial hydrocarbon employed and another organic, or mineral acid may be used together with the oxalic acid as far as necessary to give the product the acidity required for the tanning process.

The tanning process proceeds very rapidly and a solid leather showing a well marketable color is thereby produced.

25 We claim:

1. As a new composition of matter, a new form of sulfonated crude anthracene which product on hide suspended in its dilute acid

solution slowly produces a pure brown coloration.

2. As a new composition of matter, sulfonated crude anthracene, with an addition of oxalic acid which product on hide suspended in its dilute acid solution slowly produces a pure brown coloration.

3. As a new composition of matter, sulfonated crude anthracene, treated with chlorin and with an addition of oxalic acid which product on hide suspended in its dilute acid solution slowly produces a pure brown coloration.

4. The process of producing a synthetic material suitable for tanning hide which consists in treating sulfonated crude anthracene, in a practically neutral solution, with active chlorin.

5. The process of producing a synthetic material suitable for tanning hide which consists in treating sulfonated crude anthracene, in a practically neutral solution, with active chlorin and then adding oxalic acid.

In testimony whereof we have hereunto set our hands.

DR. CARL IMMERHEISER.  
HUGO WOLFF.